

# UNITED STATES PATENT OFFICE

CHARLES H. ELLIOTT AND ELMER T. McCLEARY, OF YOUNGSTOWN, OHIO, ASSIGNEES TO  
THE YOUNGSTOWN SHEET & TUBE COMPANY, OF YOUNGSTOWN, OHIO, A CORPORA-  
TION OF OHIO.

## OPEN-HEARTH STEEL PROCESS.

1,266,928.

Specification of Letters Patent. Patented May 21, 1918.

No Drawing.

Application filed July 20, 1917. Serial No. 181,887.

To all whom it may concern:

Be it known that we, CHARLES H. ELLIOTT and ELMER T. McCLEARY, citizens of the United States, residing at Youngstown, in the county of Mahoning and the State of Ohio, have invented a new and useful Open-Hearth Steel Process, of which the following is a full, clear, and exact description.

Heretofore in the manufacture of steel by 10 the open hearth process, particularly in the case of higher carbon steels, such as steel having from .2 per cent and upward of carbon, it has been common practice to take a test sample, or "preliminary test", from the 15 bath at or near the end of the heat and analyze this in the laboratory in order to ascertain whether or not the steel is in proper condition for pouring. This analysis occupies usually about thirty minutes and 20 during that time the carbon is being reduced in the bath so that when the analysis has been obtained it no longer represents the composition of the bath. Testing by fracture of a solidified sample has always been 25 used, but this is uncertain and causes many mistakes.

Furthermore, where rebarburizing is carried out by adding pig iron to the bath at the end of the heat, this addition causes a 30 violent ebullition which makes it uncertain as to how much of the carbon which is added to the bath is taken up by the steel bath and how much is lost by the excessive throwing off of gases. Consequently, it is difficult, if 35 not impossible, to obtain a specific desired carbon content in the steel where rebarburizing is carried out by additions to the bath in the furnace.

We have discovered a method of overcom- 40 ing these difficulties and we will now explain the two phases of the process as follows:

First: To overcome the decrease of the carbon content of the bath during the analysis of the test sample, we add approximately 45 sufficient silicon to the bath to prevent the oxidation of the carbon content during the period of analysis. For example, when the preliminary test sample is taken, we feed into the bath sufficient silicon pig iron to 50 supply the silicon to be burned during the ordinary period of analysis. As is well known, silicon will be attacked and burned before the carbon is attacked, and consequently when sufficient silicon is supplied to 55 the bath to last through the analysis period

the carbon will not be attacked through this period, but will remain constant.

For example, in a hundred ton bath in the open hearth, we add under a hundred pounds and preferably about fifty pounds of silicon 60 pig iron per ton of steel. The pig iron which we are employing has about the following metalloid analysis:

|            |                |    |
|------------|----------------|----|
| Silicon    | 8 per cent.    | 65 |
| Carbon     | 4 per cent.    |    |
| Phosphorus | .250 per cent. |    |
| Sulfur     | .015 per cent. |    |
| Manganese  | .80 per cent.  |    |

The silicon may, of course, be added in other forms, such as ferrosilicon, in any case 70 the silicon being added to approximately the correct amount to receive the oxidation during the analysis period and be burnt out at the end of this period while preventing the carbon from being attacked through such 75 period.

In any case the analysis of the material containing the silicon should, of course, be known, so that approximately the correct amount of silicon may be added for this 80 purpose.

The silicon addition is in such small proportion to the total bath that the carbon and other metalloids in the addition do not materially affect the metalloid contents of 85 the bath other than as to silicon.

In case the test analysis requires more than the normal time of about thirty minutes, additional silicon may be added to prevent the attacking of the carbon. In case the preliminary analysis shows that the bath requires further refining, this may be carried on, another test sample taken out and analyzed and a further addition of silicon may be sufficient to prevent attacking the carbon 95 during this new period, and so on, repeating the process until the desired analysis is reached.

If the analysis shows that the carbon content of the bath is too low, rebarburizers may 100 be added either in the furnace or ladle after tapping the heat. In any case, the operator has substantially exact knowledge of the carbon content of the bath, at the time of tapping the steel.

In carrying out our process, we preferably rebarburize the steel to bring it up to the desired carbon content by adding carbon to the steel in the ladle after tapping; for example, in the form of ferromanganese, 110

spiegeleisen, or any other desired form. The carbon may, however, be added in the bath in the form of ferromanganese or otherwise within the scope of our invention.

5 Under the second phase of the invention, we employ a silicon addition in case re-carburizing is carried out by adding pig iron or spiegel to the bath at the end of the heat in order to prevent the excessive ebullition 10 or "kick" of the metal. In this case, when the bath has been brought to the proper carbon content, using the other phase of our method or not, as desired, sufficient silicon pig or silicon carrying material is added 15 to "kill" the bath and reduce or stop the boil or ebullition. The addition of the re-carburizer is then made to the bath, the silicon of the addition burning out between the silicon addition and the addition of the re- 20 carburizer. In this case the bath may be carried down to a low carbon content, for example, .1 per cent. and is then raised to the desired content by bath addition.

Here the silicon addition prevents the violent and sudden ebullition of the bath 25 which would throw out a large and varying amount of carbon addition, and enables the per cent. of carbon addition passing into the metal to be accurately determined.

In other words, under the first phase of 30 our process, we hold in the bath the carbon already present, during the analysis period; while in the second phase we hold in the carbon then added to the bath in the carbon carrying addition.

35 In the second phase the addition may be in the form of molten pig iron from the mixer or molten spiegel added to the bath at the end of the heat before tapping, the silicon addition being made just before this 40 bath addition to prevent excessive ebullition when the bath addition is made.

The advantages of our invention will be obvious to those skilled in the art, since the operations are made more accurate and 45 worked to specification more successfully. "Off heats" may be prevented, or may be remedied by our methods.

Under the first phase, the preliminary analysis may be made just before, or just after the silicon addition. If the preliminary analysis is made after the addition, the silicon analysis will, of course, be unnecessary, as the silicon of the addition will be burned out during the taking of the analysis.

50 The amount of silicon pig added will, of course, vary with the amount of the bath and its condition. The silicon addition also serves to aid in deoxidizing the material and effecting a saving in the amount of ferromanganese, spiegeleisen or ferro-silicon in 55 case they are used. The silicon-dioxid which

will be formed also aids in cleansing the steel and having a better physical condition. The temperature of the bath will also be raised 65 by the oxidation of the silicon, thus aiding in eliminating the sulfur.

The process also enables us to tap all heats at a substantially uniform temperature since the rise in temperature is governed by the 70 amount of silicon added, a larger amount being added for a low temperature bath, and less for a higher temperature heat.

Under the second phase the "killing" of the metal aids in avoiding the formation of 75 "puddle holes" in the bottom of the furnace, which cause much expense, labor and delay.

Variations may be made in the amount of silicon addition, the kind of addition used, and other changes may be made without departing 80 from our invention.

We claim:

1. In the manufacture of open hearth steel, the steps consisting of testing the bath composition at near the end of the heat and adding silicon in conjunction therewith to retain the carbon of the bath during the 85 testing period.

2. In the manufacture of open hearth steel, the steps consisting of adding silicon to the bath in the open hearth furnace near the end of the heat, and then re-carburizing the metal, the silicon serving to hold the carbon in the bath. 90

3. In the manufacture of open hearth steel, the steps consisting of making a preliminary metalloid analysis of the bath and adding in conjunction with said analysis a proper amount of silicon to hold the carbon content of the bath substantially uniform 100 during the period of analysis.

4. In the manufacture of open hearth steel, the steps consisting of making a preliminary metalloid analysis of the bath and adding in conjunction with said analysis a proper amount of silicon to hold the carbon content of the bath substantially uniform during the period of analysis, and then re-carburizing to raise the carbon content of 105 the metal. 110

5. In the manufacture of open hearth steel, the steps consisting of making a preliminary metalloid analysis of the bath and adding in conjunction with said analysis a proper amount of silicon to hold the carbon content of the bath substantially uniform 115 during the period of analysis, tapping out the metal and then re-carburizing the metal in the ladle.

In testimony whereof, we have hereunto 120 set our hands.

CHARLES H. ELLIOTT.  
ELMER T. McCLEARY.